

## UNITED STATES PATENT OFFICE

ALBERT JEAN DUCAMP, OF VERSAILLES, FRANCE

## PROCESS FOR PREVENTING PREIGNITION IN INTERNAL COMBUSTION ENGINES

No Drawing. Original application filed March 9, 1929, Serial No. 345,878, and in France March 24, 1928.  
Divided and this application filed January 23, 1931. Serial No. 510,851.

The present application is a division from my application Serial No. 345,878 filed March 9th 1929.

The present invention has reference to processes and compositions for preventing pre-ignition in internal combustion engines.

One object of the invention is to use the lubricating oil of the engine as a carrier for introducing an anti-knock composition into the cylinders of the engine, it being understood that by an anti-knock composition is meant a composition calculated to prevent the occurrence of pre-ignition.

Another object of the invention is to use mercury cyanide to form an anti-knock composition.

As is well known, during the suction stroke of a four-stroke engine for example, the piston moves down and the walls of the cylinder, covered by a film of lubricating oil, are in contact with the in-drawn gases which are in a state of turbulence. Such contact lasts through the second or compression stroke and it is known that a certain proportion of the lubricating oil in question mixes with the fuel and burns during combustion. For example, it is generally assumed that a properly designed explosion engine will have an oil consumption, due to combustion, equal to at least one per cent by weight of its fuel consumption. Hence, if one per cent of anti-knock material be introduced into the lubricating oil, the fuel will burn in the presence of one ten thousandth part of anti-knock substance.

One way of carrying out the process consists in dissolving the anti-knock substance in a combustible or non-combustible solvent, for example in glycerine to which phenol may or may not be added and in suspending the glycerine or other solvent containing the anti-knock substance in the lubricating oil. When the lubricating oil is a mineral oil formed of hydrocarbons, free, fatty and preferably oxidized acids or alkaline or preferably alkaline-earth soaps, magnesium or calcium oleate for example, may be used as agents for suspending the glycerine in the hydrocarbons. Other suspending agents may likewise be used.

Naturally, if the lubricating oil be a fatty oil, the glycerine with its anti-knock content is suspended in the same manner which consists in considerably lowering, by means of an emulsion producing agent the inter-surface tension between the liquid containing the anti-knock substance and the lubricating oil.

For example, glycerine containing 20% by weight of mercury cyanide may be utilized and 10% by weight of said glycerine may be suspended in the lubricating oil. There will be finally 2% of anti-knock compound in the lubricating oil and if the oil burned by the engine is 2% by weight of the fuel, the percentage of mercury cyanide in terms of fuel will be 2% of 2%, i. e. .04%.

The process is particularly applicable to lubricating oils which have the property of burning at comparatively low temperatures. Such lubricating oils burn very readily during the combustion of the fuel and constitute a particularly appropriate carrier for the anti-knock compound;

I claim:

1. An anti-knock composition for use in internal combustion engines, consisting of a mercury cyanide dissolved in glycerine and suspended in the lubricating oil of the engine cylinders.

2. An anti-knock composition for use in internal combustion engines, consisting of a mercury cyanide dissolved in glycerine mixed with a fatty acid and suspended in the lubricating oil of the engine cylinders.

3. An anti-knock composition for use in internal combustion engines, consisting of a mercury cyanide dissolved in glycerine mixed with a fatty substance containing an alkali and suspended in the lubricating oil of the engine cylinders.

ALBERT JEAN DUCAMP.